

## 1

3,541,723

MOTOR FUELS CONTAINING  
MONOCARBOXYLIC ACIDS

George W. Eckert, Wappingers Falls, N.Y., assignor to  
Texaco Inc., a corporation of Delaware  
No Drawing. Filed Oct. 11, 1957, Ser. No. 689,466

Int. Cl. C10l

U.S. Cl. 44—66

6 Claims

This invention relates to a hydrocarbon fuel composition of high octane rating. More specifically, it involves the discovery that the octane rating of leaded gasoline fuels is substantially improved by the addition of carboxylic acids.

The recent increases in compression ratios of automobile engines have placed a severe strain on petroleum refiners to produce fuels having the octane rating demanded by these engines. Premium fuels at the present time have research octane ratings between 97 and 100 and it has been predicted that premium fuels will have to have octane ratings between 105 and 110 five years from now in order to satisfy the octane requirements of the high compression automotive engines predicted for that date. In order to produce premium fuels of octane ratings of 97 and above, it has been necessary for refiners to rely heavily on catalytic refining operations such as fluid catalytic cracking, catalytic reforming, alkylation and catalytic isomerization.

Catalytic cracking and catalytic reforming, which are the most widely used refining operations in the production of high octane fuels, produce substantial quantities of aromatics; catalytic cracking also produces a substantial amount of olefins. It is well-known that olefins and aromatics, although possessing high octane ratings, have a poorer response to organo-lead compounds such as tetraethyl lead than saturated aliphatic gasoline components. Accordingly, as the aromatic and olefinic content of the gasolines have increased to meet the octane levels required by modern automotive high compression engines, the lead response of the resulting fuels has diminished. Stated another way, the octane increment obtainable by the addition of an organo-lead compound decreases as the aromatic and olefin contents of the base fuel increase. The subject invention involves the discovery that the octane rating of leaded motor fuels containing a substantial concentration of high octane components, that is, aromatics, olefins and mixtures thereof, is markedly improved by the addition of a small amount of a monocarboxylic acid.

The high octane hydrocarbon motor fuel of this invention comprises high octane components including a substantial concentration of aromatic hydrocarbons, olefinic hydrocarbons or mixtures thereof, an organo-lead anti-knock agent, and a monocarboxylic acid in a concentration of at least 0.1 volume percent of the fuel.

The action of monocarboxylic acids in raising the octane rating of gasoline is characterized by several unusual features. In the first instance, the carboxylic acids appear to be ineffective in raising the octane rating of gasolines unless an organo-lead anti-knock agent, normally tetraethyl lead, is a component of the gasoline mixture.

The second unusual characteristic of the action of monocarboxylic acids in appreciating the octane rating of gasolines is the fact that equal concentrations of acids appear to cause a greater octane improvement above the 100 octane level than below the 100 octane level. For example, a 3.9 unit octane improvement on the research scale has been realized with 0.5 weight percent concentration of 2-ethylhexanoic acid in 105 octane base fuel,

## 2

whereas only a 2.3 unit improvement was realized with the same concentration of 2-ethylhexanoic acid in a base fuel having a 96.6 octane rating.

The third unusual feature of the action of monocarboxylic acids is that they appear to have substantially no effect on the octane rating of a gasoline consisting essentially of saturated aliphatic hydrocarbons even though an organo-lead anti-knock agent is present. Since organo-lead anti-knock agents exert their greatest octane appreciation in predominantly saturated paraffinic base hydrocarbon gasolines and have the least effect on the octane rating of aromatic and olefin rich gasolines, the present invention neatly complements tetraethyl lead as an octane improver. Monocarboxylic acids have their minimum effect where tetraethyl lead has its maximum effect and exert their maximum effect on octane values where tetraethyl lead has its minimum effect.

The novel fuel compositions of this invention have a minimum concentration of aromatic and/or olefin components of at least 10 volume percent. The aromatic and/or olefin components of the motor fuel of the invention can constitute as high as 100 volume percent thereof but usually fall between 20 and 20 volume percent. The minimum 10 percent concentration is necessary for monocarboxylic acids to exert a significant octane improvement.

The aromatic components of the motor fuel of the invention are generally supplied by catalytic reforming or catalytic cracking operations. Catalytic reformate is particularly high in aromatics. The olefin components of the motor fuel of the invention are derived either from thermal cracking, catalytic cracking or polymerization.

The organo-lead reagent necessary for the action of monocarboxylic acids as octane improvers is a tetraalkyl lead compound of the class known to possess anti-knock action. Tetraethyl lead is practically universally used as an anti-knock agent but other tetraalkyl lead compounds such as tetramethyl lead, tetrabutyl lead, tetraamyl lead, tetrapropyl lead, etc. are known to possess anti-knock properties and may be used in the fuel compositions of the invention in conjunction with monocarboxylic acids.

The tetraethyl lead mixtures commercially available for automotive use contain an ethylene chloride-ethylene bromide mixture as a scavenger for removing lead from the combustion chamber in the form of volatile lead halides. As is used hereafter in the examples illustrating the invention, "tetraethyl lead fluid" denotes the commercial product which comprises tetraethyl lead, ethylene chloride and ethylene bromide, the latter two reagents being present in 1.0 theory and 0.5 theory respectively, theory denoting the stoichiometric amount required for reaction with the lead content of the tetraethyl lead.

The organo-lead reagent is present in the fuel compositions of the invention in concentrations between 0.5 ml. per gallon up to the statutory limit of organo-lead reagent concentration which, at the present time, is 3 ml. per gallon in the case of automotive fuel and 4.6 ml. per gallon in the case of aviation fuel. The usual concentration of tetraethyl lead is between 1 and 3 ml. per gallon in automotive gasoline and 2-4.6 ml. per gallon in aviation gasoline.

Monocarboxylic acids which are effective in increasing the octane rating of an aromatic and/or olefin-containing gasoline in the presence of an organo-lead anti-knock agent, contain 1 to 30 carbon atoms and have the general formula: RCOOH wherein R is hydrogen or a hydrocarbyl radical containing 1 to 29 carbon atoms. Aliphatic monocarboxylic acids, cycloaliphatic monocarboxylic

acids, and aromatic monocarboxylic acids have all been found to be octane appreciators in leaded fuels containing a substantial aromatic and/or olefin content. Apparently, the action is a function of the carboxylic acid radical since aliphatic acids from formic acid up to and including behenic acid, aryl acids such as benzoic acid and cumic acid and cycloaliphatic acids have been effective in raising the octane rating of the fuel compositions of the invention.

As will be evident from the following list of monocarboxylic acids that are effective as octane appreciators in the fuel compositions of the invention, the radical attached to the carboxylic acid radical in the general formula  $\text{RCOOH}$  can be hydrogen, a saturated hydrocarbon radical, an unsaturated hydrocarbon radical, an aryl radical, an alkaryl radical, an aralkyl radical, or a cycloalkyl radical. Monocarboxylic acids that have been effective in the fuel compositions of the invention as octane improvers are the following:

Acetic acid, formic acid, propionic acid, caproic acid, 20 n-heptanoic acid, pelargonic acid, capric acid, lauric acid, myristic acid, palmitic acid, stearic acid, behenic acid, 2-ethylbutyric acid, 4-methylvaleric acid, 2-ethylhexanoic acid, cumic acid, benzoic acid, cyclohexane carboxylic acid, cinnamic acid, phenylacetic acid, oleic acid, Snodotte acids (hydrogenated fish oil fatty acids comprising mainly  $\text{C}_{10}$  to  $\text{C}_{22}$  acids), and coconut fatty acids (comprising mainly a mixture of  $\text{C}_{12}$  to  $\text{C}_{16}$  fatty acids).

Although monocarboxylic acids containing 1 to 30 carbon atoms are effective in the fuel compositions of the invention, the preferred acids contain 6 to 14 carbon atoms and are either aliphatic monocarboxylic acids or aromatic monocarboxylic acids. Monocarboxylic acids containing less than 6 carbon atoms are effective as octane improvers but have the serious drawbacks of being water-soluble, odoriferous and corrosive to metals. Preferred acids are 2-ethylhexanoic, benzoic, caprylic, capric, lauric, and myristic.

Hydroxy monocarboxylic acids such as salicylic and ricinoleic acid, halogenated carboxylic acids such as alpha-chloro-propionic acid and sulphydryl-substituted carboxylic acids such as mercapto-acetic acid, are ineffective in raising the octane rating of leaded fuels containing a substantial content of aromatics and olefins. Amino acids are too insoluble in gasoline hydrocarbons to be effective as actane appreciators. The ineffectiveness of the substituted hydrocarbon monocarboxylic acids of the types mentioned is another surprising feature of this invention.

The monocarboxylic acids must be present in the leaded aromatic and/or olefin-containing compositions of the invention in a minimum concentration of 0.1 volume percent before a significant octane appreciation is realized. With monocarboxylic acid concentrations below 0.1 volume percent, no octane improvement is obtained in leaded gasoline containing at least 10 volume percent aromatics and/or olefins. The preferred concentration of monocarboxylic acid in the fuel compositions of the invention falls between 0.2 and 1.0 volume percent with maximum octane appreciation generally being obtained at a concentration level of about 0.5 volume percent. Concentrations of monocarboxylic acids as high as 5 volume percent can be incorporated in the fuel compositions but no additional octane improvement is realized at the higher concentrations and economic considerations preclude the use of such concentrations in commercial fuel compositions.

In Table I there is shown the action of monocarboxylic acids in raising the octane rating of the leaded fuel compositions of the invention. The base gasoline to which the various acids were added in the indicated concentrations was a catalytically reformed naphtha containing 3 cc. of tetraethyl lead fluid per gallon and having an IBP of  $130^{\circ}$  F. and an end point of  $394^{\circ}$  F. The base fuel had a leaded research octane rating of 96.6 and an aromatic concentration of 48 volume percent as measured by Fluorescent Indicator Analysis (FIA) Method.

TABLE I

| Percent Acid                                                                               | Research octane numbers in 93.6 base fuel |      |      |      |      |
|--------------------------------------------------------------------------------------------|-------------------------------------------|------|------|------|------|
|                                                                                            | 0.05                                      | 0.1  | 0.25 | 0.50 | 0.75 |
| 5                                                                                          |                                           |      |      |      |      |
| Acids:                                                                                     |                                           |      |      |      |      |
| Formic                                                                                     | 97.2                                      | 97.3 | 97.5 |      |      |
| Acetic                                                                                     |                                           |      | 97.8 |      |      |
| Propionic                                                                                  | 97.4                                      | 98.0 | 97.9 |      |      |
| Caproic                                                                                    | 97.1                                      | 98.4 |      | 98.1 |      |
| n-Heptanoic                                                                                |                                           | 97.8 |      |      |      |
| Pelargonic                                                                                 |                                           | 97.8 |      |      |      |
| Capric                                                                                     |                                           | 97.2 | 97.6 | 97.6 |      |
| Lauric                                                                                     |                                           | 96.8 | 97.2 | 98.2 |      |
| Myristic                                                                                   |                                           |      | 98.0 |      |      |
| Palmitic                                                                                   |                                           |      | 97.6 |      |      |
| Stearic                                                                                    |                                           |      | 97.5 |      |      |
| Behenic                                                                                    |                                           |      | 97.4 |      |      |
| 2-ethyl butyric                                                                            |                                           |      | 97.6 |      |      |
| 4-methyl valeric                                                                           |                                           | 98.5 | 98.6 | 98.0 |      |
| 2-ethyl hexanoic                                                                           | 96.6                                      | 98.5 | 98.9 | 98.9 |      |
| $\text{C}_{10}$ acid obtained by oxidation of product of carbonylation of propylene trimer |                                           |      | 98.0 |      |      |
| Di-neopentyl acetic                                                                        |                                           |      | 98.8 |      |      |
| Neopentyl, t-butyl methyl acetic                                                           |                                           |      | 98.4 |      |      |
| Oleic                                                                                      |                                           |      | 97.5 |      |      |
| Coconut fatty acids                                                                        |                                           |      | 98.2 |      |      |
| Snodotte acids                                                                             |                                           |      | 97.5 |      |      |
| Cyclohexane carboxylic                                                                     |                                           |      | 97.9 |      |      |
| Phenyl acetic                                                                              |                                           |      | 97.9 |      |      |
| Cinnamic                                                                                   |                                           |      | 98.9 |      |      |
| Benzoic                                                                                    |                                           |      | 99.0 |      |      |

The data in the foregoing table demonstrate very clearly the effectiveness of the prescribed concentrations of hydrocarbon monocarboxylic acids in raising the octane rating of leaded gasoline having the prescribed aromatic content. The wide scope of the action of the acids is particularly significant with substantial improvement in octane rating being obtained with monocarboxylic acids containing 1-22 carbon atoms.

The data in Table I also demonstrate the necessity of employing a concentration of at least 0.1 volume percent in order to obtain any measurable octane appreciation of the leaded fuel. The addition of 0.05 volume percent of 2-ethyl hexanoic acid, one of the most effective acids, had no measurable effect on the octane rating of the base fuel, whereas almost a two unit improvement was obtained at a concentration of 0.1 volume percent of the same acid.

In Table II there is shown the action of various acids in improving the octane rating of a leaded gasoline having an octane rating of 100. The base fuel employed in Table II was a blend comprising approximately 5 percent butane, 38 percent light fluid catalytically cracked naphtha, and 57 percent catalytically reformed naphtha. The base fuel contained 3 cc. of tetraethyl lead fluid per gallon and had an aromatic content of approximately 24 volume percent as measured by FIA Method. The 100 octane base fuel had an IBP of  $98^{\circ}$  F. and an end point of  $363^{\circ}$  F.

TABLE II

| Volume percent of acid in fuel    | Research octane values in 100 octane gasoline |       |       |       |       |
|-----------------------------------|-----------------------------------------------|-------|-------|-------|-------|
|                                   | 0.1                                           | 0.25  | 0.50  | 1.00  | 2.00  |
| 55                                |                                               |       |       |       |       |
| Acids:                            |                                               |       |       |       |       |
| Lauric                            | 99.9                                          | 100.1 | 100.4 | 101.8 | 100.9 |
| Capric                            | 99.4                                          | 99.6  | 100.5 | 101.3 |       |
| Neopentyl, t-butyl, methyl acetic | 99.9                                          | 100.4 | 100.9 | 101.2 |       |
| Cumic                             | 99.7                                          | 99.7  | 100.7 | 101.4 |       |
| Cyclohexane carboxylic            | 100.3                                         | 100.8 | 101.9 | 100.4 | 98.6  |
| 2-ethylhexanoic                   | 101.2                                         | 102.1 | 102.0 |       |       |
| Benzoic                           | (1)                                           | 100.9 |       |       |       |

<sup>1</sup> 0.2 percent.

In Table III there is shown the effectiveness of three different types of monocarboxylic acids, namely, 2-ethylhexanoic acid, cyclohexane carboxylic acid, and benzoic acid in improving the octane rating of a 105 octane gasoline containing 3 cc. of tetraethyl lead fluid per gallon and comprising approximately 10 percent butane, 40 percent isobutaneisobutylene alkylate, 10 percent pentenes from a liquid catalytically cracked naphtha and 40 percent heavy platformate. The 105 research octane base fuel had an aromatic content of approximately 32 percent and an olefin content of approximately 12 percent.

TABLE III

| Volume percent of acid | Research octane values—<br>105 octane gasoline |       |       |       |
|------------------------|------------------------------------------------|-------|-------|-------|
|                        | 0.1                                            | 0.25  | 0.50  | 1.00  |
| Acids:                 |                                                |       |       |       |
| Cyclohexane carboxylic | 105.8                                          | 106.5 | 107.8 | 106.7 |
| 2-ethylhexanoic        | 107.6                                          | 109.2 |       |       |
| Benzoic                | 108.0                                          | 107.9 | 108.6 | 107.4 |

The octane improvements in the 105 octane base fuel resulting from the addition of the 0.1 to 1.0 volume percent acid are dramatic. The 3.9 unit improvement in research octane value obtained by the addition of 0.5 volume percent 2-ethylhexanoic acid, the 3.6 unit improvement resulting from the same concentration of benzoic acid, and the 2.8 unit improvement resulting from the presence of the same concentration of cyclohexane carboxylic acid are outstanding. Prior to this invention, octane improvements of this magnitude at the 105 octane level were considered impossible to attain. It is also significant that greater octane improvement is obtained by equivalent concentrations of the benzoic, 2-ethylhexanoic and cyclohexane carboxylic acid in the 105 octane base fuel than in the 96.6 and 100 octane base fuels of Tables I and II, respectively.

10

15

20

25

TABLE V

| Base fuel                                                 | Research octane number                |                                       |
|-----------------------------------------------------------|---------------------------------------|---------------------------------------|
|                                                           | With 3<br>cc./gal.<br>Clear TEL fluid | With 3<br>cc./gal.<br>Clear TEL fluid |
| Base fuel D                                               | 84.3                                  | 97.8                                  |
| Base fuel D plus 0.5 vol. percent 2-ethylhexanoic<br>Acid | 84.3                                  | 98.1                                  |
| Base fuel E                                               | 69.2                                  | 86.9                                  |
| Base fuel E plus 0.5 vol. percent 2-ethylhexanoic<br>acid | 69.7                                  | 86.8                                  |

The data in Table V show that in predominantly saturated aliphatic gasoline, the addition of the hydrocarbon monocarboxylic acid has substantially no effect on the octane rating of the fuel even in the presence of the organo-lead anti-knock agent. It is noteworthy that it is in such fuels that tetraethyl lead is particularly effective in increasing the octane rating.

In Table VI it is shown that both the research and motor octane ratings of a commercial gasoline containing 3 cc. of tetraethyl lead fluid per gallon, and comprising approximately 26 percent aromatic hydrocarbons, 14 percent olefins and 60 percent saturated hydrocarbons are significantly improved by the addition of the prescribed amounts of 2-ethylhexanoic acid and benzoic acid.

TABLE VI

|                                                      | Research<br>octane<br>No. | Motor<br>octane<br>No. |
|------------------------------------------------------|---------------------------|------------------------|
| Base fuel                                            | 97.0                      | 88.5                   |
| Base fuel plus 0.1 vol. percent 2-ethylhexanoic acid | 97.4                      | 89.5                   |
| Base fuel plus 0.2 vol. percent 2-ethylhexanoic acid | 97.5                      | 89.7                   |
| Base fuel plus 0.5 vol. percent 2-ethylhexanoic acid | 98.2                      |                        |
| Base fuel plus 0.1 vol. percent benzoic acid         | 97.7                      | 89.5                   |
| Base fuel plus 0.2 vol. percent benzoic acid         | 98.0                      | 90.0                   |

In Table IV there is shown the necessity of an organo-lead anti-knock agent in the aromatic and/or olefin-containing fuel in order for the monocarboxylic acid to effect octane improvement of the fuel. Base Fuel A employed in Table IV was the catalytically reformed naphtha employed in Table I.

TABLE IV

|                                                           | Research octane<br>numbers            |                                       |
|-----------------------------------------------------------|---------------------------------------|---------------------------------------|
|                                                           | With 3<br>cc./gal.<br>Clear TEL fluid | With 3<br>cc./gal.<br>Clear TEL fluid |
|                                                           |                                       | Base fuel A                           |
| Base fuel A plus 0.5 vol. percent 2-ethylhexanoic<br>acid | 87.4                                  | 98.9                                  |
| Base fuel A plus 0.5 vol. percent benzoic acid            | 88.0                                  | 98.5                                  |
| Pentene-2                                                 | 95.1                                  | 98.6                                  |
| Pentene-2 plus 0.5 vol. percent benzoic acid              | 94.6                                  | 99.4                                  |
| Heavy C.R. Naphtha                                        | 103.4                                 | 105.6                                 |
| Heavy C.R. Naphtha plus 0.5 vol. percent benzoic<br>acid  | 102.9                                 | 108.0                                 |

The data in Table IV indicate that the prescribed concentration of monocarboxylic acid in the absence of an organo-lead anti-knock agent either has no significant effect on the octane rating of the resulting fuel, or actually slightly lowers the octane rating.

The data in Table V demonstrate the ineffectiveness of hydrocarbon monocarboxylic acids in raising the octane rating of saturated aliphatic hydrocarbons in the gasoline boiling range. Base Fuel D in Table V consists essentially of 2,4-dimethylpentane; Base Fuel E is a light straight run naphtha having a boiling point range of 94° F. to 207° F.

In Table VII there is compared the action of monocarboxylic acids on the octane ratings of three different blends of high octane gasoline components. The aromatic gasoline blend had a boiling point range of 228 to 378° F. and comprised 84 percent aromatics, 15 percent saturated aliphatic hydrocarbons and 1 percent olefinic hydrocarbons. Olefinic gasoline blend A consists essentially of a mixture of dimers and trimers of propylene having a boiling point range of 102–430° F. Olefinic gasoline blend B comprised 50 percent isoctene and 50 percent isohexene. The isoparaffinic gasoline blend comprised 10 percent isopentane, 5 percent n-heptane and 85 percent isoctane.

Table VII

|                                                                         | Research octane numbers<br>with 3 cc./gal. TEL fluid |
|-------------------------------------------------------------------------|------------------------------------------------------|
| Aromatic gasoline                                                       | 108.3                                                |
| Aromatic Gasoline + 0.5 vol. percent benzoic acid                       | 110.6                                                |
| Aromatic gasoline + 0.5 vol. percent 2-ethylhexanoic<br>acid            | 110.0                                                |
| Olefinic gasoline blend A                                               | 98.6                                                 |
| Olefinic gasoline blend A + 0.5 vol. percent benzoic<br>acid            | 99.6                                                 |
| Olefinic gasoline blend B                                               | 100.4                                                |
| Olefinic gasoline blend B + 0.5 vol. percent benzoic<br>acid            | 101.1                                                |
| Olefinic gasoline blend B + 0.5 vol. percent 2-ethylhexanoic<br>acid    | 101.3                                                |
| Isoparaffinic gasoline blend                                            | 105.3                                                |
| Isoparaffinic gasoline blend + 0.5 vol. percent benzoic<br>acid         | 105.4                                                |
| Isoparaffinic gasoline blend + 0.5 vol. percent 2-ethylhexanoic<br>acid | 105.1                                                |

The data in Table VII demonstrate clearly the effectiveness of monocarboxylic acids in raising the octane ratings of leaded aromatic and olefinic gasolines and the ineffectiveness of the same acids in improving the octane ratings of a leaded isoparaffinic gasoline. These data indicate clearly that the gasoline blend must have an aromatic and/or olefin content above about 10 volume percent in order for the monocarboxylic acids to act as octane improvers.

In Table VIII, data are presented to show the ineffectiveness of hydroxy monocarboxylic acids, halo-substituted monocarboxylic acids, and mercapto-substituted monocarboxylic acids in raising the octane rating of leaded gasoline. The base fuel employed in Table VIII was the catalytically reformed naphtha described in connection with the data presented in Table I. This base fuel had an aromatic concentration of 48 volume percent and contained 3 cc. of tetraethyl lead fluid per gallon.

Table VIII

|                                                     | Research octane numbers |
|-----------------------------------------------------|-------------------------|
| Base fuel                                           | 96.6                    |
| Base fuel+0.5 v. percent ricinoleic acid            | 96.6                    |
| Base fuel+0.5 v. percent salicylic acid             | 96.6                    |
| Base fuel+0.5 v. percent monochloroacetic acid      | 87.0                    |
| Base fuel+0.5 v. percent heptafluorobutyric acid    | 89.3                    |
| Base fuel+0.5 v. percent 2-bromohexanoic acid       | 96.3                    |
| Base fuel+0.5 v. percent alpha-chloropropionic acid | 94.0                    |
| Base fuel+0.5 v. percent mercaptoacetic acid        | 96.0                    |

In addition to the hydrocarbon monocarboxylic acids, halo-monocarboxylic acids and mercapto-monocarboxylic acids shown to be ineffective in Table VIII, amino acids are unable to exert any positive action in raising the octane rating of leaded fuels containing the requisite aromatic and/or olefin content because of their insolubility in gasoline hydrocarbons.

Obviously, many modifications and variations of the invention as hereinbefore set forth may be made without departing from the spirit and scope thereof and, therefore, only such limitations should be imposed as are indicated in the appended claims.

I claim:

1. A hydrocarbon fuel in the gasoline boiling range containing an organo-lead anti-knock agent, high octane components selected from the group consisting of olefinic

hydrocarbons, aromatic hydrocarbons and mixtures thereof in a concentration of at least about 10 volume percent of said fuel and an aromatic monocarboxylic acid containing up to 30 carbon atoms in a concentration between 0.1 and 5.0 volume percent, said amount being sufficient to effect substantial improvement of the octane rating of said organo-lead-containing hydrocarbon fuel.

2. A hydrocarbon fuel according to claim 1 in which said aromatic monocarboxylic acid is a benzene monocarboxylic acid.

3. A hydrocarbon fuel according to claim 1 in which said aromatic monocarboxylic acid is benzoic acid.

4. A hydrocarbon fuel according to claim 1 in which said aromatic monocarboxylic acid is phenylacetic acid.

5. A hydrocarbon fuel according to claim 1 in which said aromatic monocarboxylic acid is cinnamic acid.

6. A hydrocarbon fuel composition according to claim 1 in which said aromatic monocarboxylic acid is cuminic acid.

#### References Cited

##### UNITED STATES PATENTS

|           |         |             |         |
|-----------|---------|-------------|---------|
| 2,125,448 | 8/1938  | Johnson     | 44—66 X |
| 2,667,408 | 1/1954  | Kleinholz   | 44—66 X |
| 1,692,784 | 11/1928 | Orelup      | 44—66   |
| 2,426,709 | 9/1947  | Roddy       | 44—66 X |
| 2,360,585 | 10/1944 | Ross et al. | 44—80   |

##### FOREIGN PATENTS

|         |        |                |
|---------|--------|----------------|
| 277,326 | 1/1929 | Great Britain. |
| 599,222 | 3/1948 | Great Britain. |
| 640,311 | 7/1928 | France.        |

##### OTHER REFERENCES

"Improved Motor Fuels Through Selective Blending,"  
35 Wagner et al., Paper Presented Before American Petroleum Institute Nov. 7, 1941.

"Aviation Gasoline Manufacture," by Van Winkle,  
McGraw-Hill Book Co. Inc., 1944, 1st edition, pp. 199—204.

PATRICK P. GARVIN, Primary Examiner

Y. H. SMITH, Assistant Examiner

U.S. Cl. X.R.

45 44—69